



US005278020A

**United States Patent [19]**

Grushkin et al.

[11] Patent Number: **5,278,020**[45] Date of Patent: **Jan. 11, 1994****[54] TONER COMPOSITION AND PROCESSES THEREOF**

[75] Inventors: **Bernard Grushkin**, Pittsford, N.Y.; **Guerino G. Sacripante**, Oakville, Canada

[73] Assignee: **Xerox Corporation**, Stamford, Conn.

[21] Appl. No.: **936,471**

[22] Filed: **Aug. 28, 1992**

[51] Int. Cl.<sup>5</sup> ..... **G03C 5/00**

[52] U.S. Cl. ..... **430/137; 430/109;**  
**430/110; 430/111; 430/138**

[58] Field of Search ..... **430/109, 110, 111, 137,**  
**430/138**

**[56] References Cited****U.S. PATENT DOCUMENTS**

- 4,797,339 1/1989 Maruyama et al. ..... 430/109  
4,876,313 10/1989 Lorah ..... 525/281  
4,983,488 1/1991 Tan et al. ..... 430/137  
4,996,127 2/1991 Hasegawa et al. ..... 430/109  
5,037,716 8/1991 Moffat ..... 430/109  
5,139,915 8/1992 Moffat et al. ..... 430/110

**OTHER PUBLICATIONS**

Ricoh RTU Spring '92, Nippon Carbide '127 Associated  
Particles.

Primary Examiner—John Kight, III

Assistant Examiner—Shelley A. Dodson

*Attorney, Agent, or Firm*—John L. Haack; Eugene O. Palazzo

**[57] ABSTRACT**

A toner composition and processes for the preparation thereof comprising the steps of: (i) preparing a latex emulsion by agitating in water a mixture of a nonionic surfactant, an anionic surfactant, a first nonpolar olefinic monomer, a second nonpolar diolefinic monomer, a free radical initiator and a chain transfer agent; (ii) polymerizing the latex emulsion mixture by heating from ambient temperature to about 80° C. to form nonpolar olefinic emulsion resin particles of volume average diameter from about 5 nanometers to about 500 nanometers; (iii) diluting the nonpolar olefinic emulsion resin particle mixture with water; (iv) adding to the diluted resin particle mixture a colorant or pigment particles and optionally dispersing the resulting mixture with a homogenizer; (v) adding a cationic surfactant to flocculate the colorant or pigment particles to the surface of the emulsion resin particles; (vi) homogenizing the flocculated mixture at high shear to form statically bound aggregated composite particles with a volume average diameter of less than or equal to about 5 microns; (vii) heating the statically bound aggregate composite particles to form nonpolar toner sized particles; (viii) optionally halogenating the nonpolar toner sized particles to form nonpolar toner sized particles having a halopolymer resin outer surface or encapsulating shell; and (ix) isolating the nonpolar toner sized composite particles.

**30 Claims, No Drawings**

## TONER COMPOSITION AND PROCESSES THEREOF

### BACKGROUND OF THE INVENTION

This invention is generally directed to toner and developer compositions, and, more specifically, the present invention is directed to toner compositions and processes for the preparation of toner compositions. In one embodiment, there are provided in accordance with the present invention in situ processes for the preparation of toner compositions with average volume particle sizes equal to, or less than about 10 micrometers in embodiments without resorting to classification. The resulting toners can be selected for known electrophotographic imaging and printing processes, including color processes, and lithography. In an embodiment, the present invention is directed to a process for preparing a toner comprised of composite particles comprised of primary particles comprised of a nonpolar copolymer resin, secondary particles comprised of a pigment, wherein the secondary particles reside substantially on the surface of the primary particles and wherein the composite particles may have chemically modified outer surfaces and an average diameter of about 1 to 10 micrometers. In embodiments, the process of the present invention comprises preparing a latex emulsion by agitating a mixture of nonpolar olefins such as styrene and butadiene in an aqueous medium containing a mixture of nonionic and anionic surfactants, a chain transfer agent and a free radical initiator, and polymerizing the mixture by heating to form nonpolar olefinic resin particles in water comprised of, for example, poly(styrene-butadiene); thereafter adding and dispersing pigment particles with the nonpolar olefinic resin particles and flocculating the mixture by the addition of a cationic surfactant; homogenizing the flocculated mixture to form statically bound resin and pigment particle aggregates of from less than about 5 micrometers; heating and thereby fusing the pigment and resin particle aggregate mixture to form composite nonpolar toner sized particles of from about 3 to about 10 micrometers; optionally, chemically modifying the toner surface with, for example, chlorine gas to transform the olefinic resin present on the outer surface of the composite toner particle to, for example, a chlorinated poly(styrene butadiene) species poly(styrene-butadiene-dichloro butene); and isolating the toner particles by concentrating, washing and drying. The toner and developer compositions of the present invention can be selected for electrophotographic, especially xerographic imaging and printing processes, including color processes.

In reprographic technologies, such as xerographic and ionographic devices, toners with small average volume diameter particle sizes of from about 5 microns to about 20 microns are utilized. Moreover, in some xerographic technologies, such as the high volume Xerox Corporation 5090<sup>TM</sup> copier-duplicator, high resolution characteristics and low image noise are highly desired, and can be readily attained utilizing small sized toners with average volume particle of less than 11 microns and preferably less than about 7 microns and with narrow geometric size distribution (GSD) of less than about 1.6, preferably less than about 1.4, and more preferably less than about 1.3. Additionally, in some xerographic systems wherein process color is required such as pictorial color applications, small particle size colored toners of less than 9 microns

and preferably less than about 7 microns are highly desired to avoid paper curling. Paper curling is especially observed in pictorial or process color applications wherein three to four layers of toners are transferred and fused onto paper. During the fusing step, moisture is driven off from the paper due to the high fusing temperatures of from about 130 to 160 degrees centigrade applied to the paper from the fuser. Where only one layer of toner is present such as in black or highlight xerographic applications, the amount of moisture driven off during fusing is re-absorbed proportionally by paper and the resulting print remains relatively flat with minimal curl. In pictorial color process applications wherein three to four colored toner layers are present, a thicker toner plastic level present after the fusing step inhibits the paper from sufficiently absorbing the moisture lost during the fusing step, and image paper curling results. Since surface area of particle size is inversely proportional to particle size, it is preferable to use small toner particle sizes of less than 9 microns and preferably less than about 7 microns and with higher pigment loading such that the mass of toner layers deposited onto paper is reduced to obtain the same quality of image and resulting in a thinner plastic toner layer onto paper after fusing, and hence, minimizing or avoiding paper curling. Toners prepared in the instant invention with lower fusing temperatures such as from about 100 to about 140 degrees centigrade help to avoid paper curl. Lower fusing temperatures minimizes the loss of moisture from paper, thereby reducing or eliminating paper curl. Furthermore, in process color applications and especially in pictorial color applications, high gloss is necessary, as well as high projection efficiency properties with transparency images.

Numerous processes are known for the preparation of toners, such as, for example, conventional processes wherein a resin is melt kneaded or extruded with a pigment, micronized and pulverized to provide toner particles with an average volume particle diameter of from about 7 microns to about 20 microns and with broad geometric size distribution of from about 1.4 to about 1.7. In such processes it is usually necessary to subject the aforementioned toners to a classification procedure such that the geometric size distribution of from about 1.2 to about 1.6 are attained. However, in the aforementioned conventional process, low toner yields after classifications may be obtained and dependent on the average volume particle sizes of said toner. Generally, during the preparation of toners with average particle size diameters of from about 11 microns to about 15 microns, toner yields range from about 70 percent to about 85 percent after classification. Additionally, during the preparation of smaller sized toners with particle sizes of from about 7 microns to about 11 microns, lower toner yields are obtained after classification, such as from about 50 percent to about 70 percent. With the processes of the present invention in embodiments, small average particle sizes of from about 3 microns to about 9, and preferably 7 microns are attained without resorting to classification processes, and wherein high toner yields are attained such as from about 90 percent to about 98 percent in embodiments. Additionally, toners prepared by conventional processes must not readily aggregate or block during manufacturing, transport or storage prior to use in electrophotographic systems and must exhibit low temperature fusing properties in order to minimize fuser energy

requirements. Accordingly, conventional toner resins are restricted to having exhibit glass transition temperatures of greater than about 55 degrees centigrade and preferably of about 60 degrees centigrade to satify caking or blocking requirements. Toner caking or blocking is known in the art and refers to the minimum temperature necessary for toner aggregation to occur over an extended period of time, such as from about 24 hours to 48 hours. The caking or blocking temperature requirement of a toner should be greater than about 55 degrees centigrade and preferably greater than about 60 degrees centigrade, in order to avoid toner aggregation in storage or use prior to fixing a powdered toner image to a receiver sheet. This blocking requirement restricts the toner fusing properties of from about 135 degrees centigrade to about 160 degrees centigrade. In process color or pictorial applications, wherein low paper curl is a requirement, low toner fusing properties are desired such as less than about 140 degrees centigrade and preferably less than 110 degrees centigrade such that moisture evaporation or removal from paper is minimized or preferably avoided. With the toners of this invention, the toners fuse at lower temperatures than conventional toners, such as from about 110 to about 150 degrees centigrade, thereby reducing the energy requirements of the fuser and more importantly resulting in lower moisture driven off from the paper during fusing, and hence lowering or minimizing paper curling. For the toners of this invention, the blocking and fusing properties of the toners are disintegrated by the chemical surface process of halogenating the toner surface. During the process for the preparation of the toner of this invention, the polymerized primary emulsion resin such as poly (styrene-butadiene) exhibits a glass transition temperature of from about 40 degrees centigrade to about 50 degrees centigrade and thermal properties amenable to achieve the low fusing properties such as from about 110 degrees centigrade to about 140 degrees centigrade, and after a flocculation and aggregation fusing process and during, for example, the chlorination step, the outer surface of the toner resin surface is chemically transformed from poly(styrene-butadiene) to chlorinated poly(styrene-butadiene) such that the outer surface of the toner resin composite has a glass transition of from about 55 degrees centigrade to about 60 degrees centigrade necessary for the blocking requirement. This latter chemical surface treatment step allows one to separate toner blocking requirements from fusing requirements and results in low fusing toners of from about 110 degrees centigrade to about 140 degrees centigrade which are necessary to minimize or eliminate paper curling. That is by lowering the fusing temperature range to about 100° to 140° C. a reduction or elimination in paper curl is achieved. In addition, by the toner particle preparation process of this invention, small particle size toners of from about 3 microns to about 7 microns are prepared with high yields as from about 90 percent to about 98 percent by weight of all toner starting material ingredients.

Additionally, other processes such as and including encapsulation, coagulation, coalescence, suspension polymerization, or semi-suspension and the like, are known, wherein the toners are obtained by in situ one pot methods. Moreover, encapsulated toners are known wherein a core comprised of pigment and resin is encapsulated by a shell, and wherein the toner melt rheological properties are separated wherein a core material provides low fusing properties such as from about 100

to 125 degrees centigrade, and an encapsulating shell provides necessary blocking properties for particle stability prior to fusing. However, it is known that encapsulated toners do not provide high gloss due to high surface tension, high glass transition and high melting temperatures of the shell, and also result in poor projection efficiency due to the difference in refractive index between the shell and core resulting in light scattering. Other in situ toners prepared by suspension, coagulation, coalescence, are known, wherein the toners are comprised of substantially similar composition to conventional toners with, in some cases, having surfactants or surface additives on the toner surface prepared by various processes. Although, these latter aforementioned toners are amenable to high gloss, high projection efficiency, and small particle size toners, their fusing performances are restricted to the thermal properties of the toner, such as glass transition (Tg), in that the toners must satisfy blocking requirements and hence are restricted to glass transitions of above 55 degrees centigrade and therefore fusing temperatures of from about 135 to about 160 degrees centigrade, and have inferior paper curl properties for process color applications. By the processes of the instant invention, toner melt rheological properties are separated in that a chemical halogenation process increases the glass transition of the outer surface of the toner composite resin of from about 45 to 55 degrees centigrade to about 55 to 60 degrees centigrade, hence providing required blocking properties and low fusing temperatures of from about 110 degrees centigrade to about 140 degrees centigrade necessary for minimizing or avoiding paper curling.

In the embodiments of the instant invention a process for the preparation of a nonpolar composite particle toner composition is disclosed comprising the steps of: (i) preparing a latex emulsion by agitating in water a mixture of nonionic surfactant such as polyethylene glycol or polyoxyethylene glycol nonyl phenyl ether, an anionic surfactant such as sodium dodecyl sulfonate or sodium dodecyl benzenesulfonate, a first nonpolar olefinic monomer such as styrene, acrylate or methacrylate, a second nonionic nonpolar diolefinic monomer such as butadiene or isoprene; (ii) polymerizing the reaction mixture by heating from ambient temperature to about 80° C. the olefinic and diolefinic monomers to nonpolar olefinic emulsion sized particles of from about 5 nanometers to about 500 nanometers in average volume diameter; (iii) diluting the nonpolar olefinic emulsion resin mixture with water from about 50% solids to about 15% solids; (iv) adding to the mixture a colorant or pigment particles of from about 3 percent to about 15 percent by weight of toner and optionally dispersing the resulting mixture by dispersing utilizing a Brinkman or IKA homogenizer; (v) adding a cationic surfactant such as dialkylbenzene dialkylammonium chloride and the like thereby effecting flocculation of the colorant or pigment particles with emulsion resin particles; (vi) homogenizing the flocculated resin-pigment mixture at from about 2000 to about 6000 revolution per minute to form high shear statically bound aggregate composite particles of less than about 5 microns in volume average diameter; (vii) heating the statically bound aggregate composite particles of from about 60 degrees centigrade to about 95 degrees centigrade and for a duration of about 60 minutes to about 600 minutes to form nonpolar toner sized particles of from about 3 microns to about 9 microns in volume average diameter; (viii) optionally halogenating the nonpolar toner sized particles with a

halogen, for example, chlorine gas to chemically transform the nonpolar olefinic moieties of the resin present on the outer surface of the toner resin to chlorine containing hydrocarbon moieties; and (ix) isolating the nonpolar toner sized composite particles by washing, filtering and drying thereby providing a nonpolar composite particle toner composition. Flow additives to improve flow characteristics may then optionally be employed such as Aerosils or silicas, and the like, of from about 0.1 to about 10 percent by weight of the toner.

In a patentability search there is illustrated in U.S. Pat. No. 4,996,127 a toner of associated particles of secondary particles comprising primary particles of a polymer having acidic or basic polar groups and a coloring agent. The polymers selected for the toners of the '127 patent can be prepared by an emulsion polymerization method, see, for example, columns 4 and 5. In column 7 of the '127 patent it is indicated that the toner can be prepared by mixing the required amount of coloring agent and optional charge additive with an emulsion of the polymer having an acidic or basic polar group obtained by emulsion polymerization as indicated in column 3. Additionally, note column 9, line 50 to 55, wherein polar monomers such as acrylic acid in the emulsion resin is necessary, and note Comparative Example 1, column 9, lines 50 to 55 wherein toner preparation is not obtained without the use of a polar group such as acrylic acid. The present invention is directed to an improved process wherein the emulsion monomers or resultant resin particles do not contain acidic or basic groups, and toner particles are obtained without the use of polar acidic groups such as acrylic acid, thereby reducing toner humidity sensitivity. Additionally, with processes of the instant invention, halogenation, for example, chlorination of the outer surface of the composite particles provides an improvement in blocking characteristics, and hence enhances the minimum fix temperature of the toner.

Illustrated in U.S. Pat. No. 4,797,339, is a toner composition comprised of an inner layer comprising a resin ion complex having a coloring agent, a charge enhancing additive and pigment dispersed therein, and an outer layer containing a flowability imparting agent. Note column 2 and 3, wherein the ion complex resin is comprised of an acidic emulsion copolymer resin and basic emulsion resin comprised of styrene acrylates containing acidic or basic polar groups similar to the '127 patent.

U.S. Pat. No. 4,983,488 discloses a process for the preparation of toners by the polymerization of a polymerizable monomer dispersed by emulsification in the presence of a colorant and/or a magnetic powder to prepare a principal resin component and then effecting coagulation of the resulting polymerization liquid in such a manner that the particles in the liquid after coagulation have diameters suitable for a toner. It is indicated in column 9 of this patent that coagulated particles of 1 to 100 micrometers in diameter, and particularly 3 to 70 micrometers in diameter, are obtained. It is also indicated in column 4, lines 60 to 65, that the glass transition of the emulsion resin should be above 50 degrees centigrade, and when the glass transition is too low, caking resistance, that is resistance to blocking, tends to decrease and if the glass transition is too high the fixing property tends to be poor. The toners of the instant invention differ from the reference toners in that the process is simple and does not utilize coagulating

agents. Moreover, emulsion resins with relatively lower glass transition of about 40 to 45 degrees centigrade are used, and resistance to caking is avoided by the halogenation process of the toner surface wherein the glass transition is raised to about 50 to about 55 degrees centigrade, hence caking, blocking or undesired aggregation of toner particles is avoided and low fixing temperatures are maintained as well as excellent triboelectric characteristics, high gloss, and low humidity sensitivity.

Copending application U.S. Ser. No. 07/767,454, filed Sep. 30, 1991, the disclosure of which is totally incorporated herein by reference, discloses an in situ suspension process for a toner comprised of a core comprised of a resin, pigment and optionally charge control agent and coated thereover with a cellulosic material. Another patent of interest is copending U.S. Ser. No. 07/695,880, filed May 6, 1991 entitled 'Toner Compositions', the disclosure of which is totally incorporated herein by reference, discloses low melt toner particles prepared by conventional comminution processes that are halogenated to form encapsulated toner particles with a higher melting halopolymer shell.

Additionally, U.S. Pat. No. 4,876,313, discloses an improved core and shell polymers having an alkali-insoluble core and an alkali-soluble shell which polymers are prepared by emulsion polymerization of the core-shell polymers utilizing compounds which chemically graft the core and shell polymers together.

Documents disclosing toner compositions with charge control additives include U.S. Pat. Nos. 3,944,493; 4,007,293; 4,079,014; 4,394,430; and 4,560,635 which illustrates a toner with a distearyl dimethyl ammonium methyl sulfate charge additive. These toners are prepared, for example, by the usual known jetting, micronization, and classification processes. Toners obtained with these processes generally possess a toner volume average diameter of form between about 10 to about 20 microns and are obtained in yields of from about 85 percent to about 98 percent by weight of starting materials without classification procedure.

There is a need for black or colored toners wherein small particle sizes of less than or equal to 7 microns in volume diameter. Furthermore, there is a need for colored toner processes wherein the toner synthetic yields are high, such as from about 90 percent to about 100 percent while avoiding or without resorting to classification procedures. In addition, there is also a need for black and colored toners that are non-blocking, such as from about 55 to about 60 degrees centigrade, of excellent image resolution, non-smearing and of excellent triboelectric charging characteristics. Moreover, there is a need for black or colored toners with: low fusing temperatures, of from about 110 degrees centigrade to about 150 degrees centigrade; of high gloss properties such as from about 50 gloss units to about 85 gloss units; of high projection efficiency, such as from about 75 percent to about 95 percent efficiency or more, and result in minimal or no paper curl.

#### SUMMARY OF THE INVENTION

It is an object of the present invention to provide toner with many of the advantages illustrated herein.

In another object of the present invention there are provided emulsion aggregation processes for the preparation of composite nonpolar toner particle compositions wherein micronizing, jetting, and classification can in embodiments be avoided.

In yet another object of the present invention there are provided toner compositions with small particle size of, for example, from about 1 to about 7 microns in average volume diameter.

In another object of the present invention there are provided composite nonpolar toner compositions of high yields of from about 90 percent to about 100 percent by weight of toner and without resorting to classification.

In yet another object of the present invention there are provided toner compositions with low fusing temperature of from about 110 degrees centigrade to about 150 degrees centigrade and of excellent blocking characteristics of more than about 55 degrees centigrade to about 60 degrees centigrade.

Another object of the present invention there are provided toner compositions with high gloss such as from about 45 gloss units to about 85 gloss units.

Moreover, in another object of the present invention there are provided toner compositions with high projection efficiency such as from about 75 to about 95 percent efficiency.

It is a further object of the present invention there are provided toner compositions which result in low paper curl.

Another object of the present invention resides in providing emulsion aggregation processes for composite nonpolar toner compositions by coalescing or fusing statically bound aggregates comprised of primary nonpolar resin emulsion particles and pigment particles and wherein the resulting toner composites possess an average diameter of from between about 3 to 15, and preferably from between about 3 to about 7 microns.

Also, in another object of the present invention there are provided developer compositions with composite nonpolar toner particles obtained by the processes illustrated herein, carrier particles, and optional enhancing additives or mixtures of these additives.

Another object of the present invention resides in the formation of toners which will enable the development of images in electrophotographic imaging apparatuses, which images have substantially no background deposits thereon, and are of excellent resolution; and further, such toner compositions can be selected for high speed electrophotographic apparatuses, that is those exceeding 70 copies per minute.

In embodiments, the present invention is directed to processes for the preparation of composite nonpolar toner compositions comprised, for example, of primary nonpolar resin particles, secondary pigment particles, and optional charge enhancing additives comprised of, for example, chromium salicylates, quaternary ammonium hydrogen bisulfates, tetraalkyl ammonium sulfonate, and the like. More specifically, the present invention in one embodiment is directed to emulsion aggregation processes for the preparation of nonpolar composite particle toner composition comprising the steps of: (i) preparing a latex emulsion by agitating in water a mixture of nonionic surfactant such as polyethylene glycol or polyoxyethylene glycol nonyl phenyl ether, an anionic surfactant such as sodium dodecyl sulfonate or sodium dodecyl benzenesulfonate, a first nonpolar olefinic monomer such as styrene, acrylate or methacrylate, a second nonpolar diolefinc monomer such as butadiene or isoprene; (ii) polymerizing the reaction mixture by heating from ambient temperature to about 80° C. the olefinic and diolefinc monomers to form

nonpolar olefinic copolymer resin particles sized from about 5 nanometers to about 500 nanometers in volume average diameter; (iii) diluting the nonpolar olefinic emulsion copolymer resin mixture with water from about 50% solids to about 15% solids; (iv) and adding to the mixture colorant or pigment particles of from about 3 percent to about 15 percent by weight of toner and optionally dispersing the mixture by dispersing utilizing a Brinkman or IKA homogenizer; (v) thereafter adding a cationic surfactant such as dialkylbenzene dialkylammonium chloride and the like thereby effecting flocculation of the colorant or pigment particles with emulsion resin; (vi) homogenizing the flocculated mixture at from about 2,000 to about 6,000 revolution per minute to form statically bound aggregate composite particles of less than about 5 microns in volume average diameter; (vii) heating the statically bound aggregate composite particles of from about 60 degrees centigrade to about 95 degrees centigrade and for a duration of about 60 minutes to about 600 minutes to form nonpolar toner sized particles of from about 3 microns to about 9 microns in volume average diameter; (viii) halogenating the nonpolar toner sized particles with for example chlorine gas to chemically transform the nonpolar olefinic moieties of the resin present on the outer surface of the toner composite to chlorine moieties; and (ix) isolating the nonpolar toner sized particles by washing, filtering and drying thereby providing a nonpolar composite particle toner composition. Flow additives to improve flow characteristics and charge additives to improve charging characteristics may then optionally be employed such as Aerosils or silicas, and the like, of from about 0.1 to about 10 percent by weight of the toner.

Illustrative examples of the nonionic monomers useful in the instant invention, include a number of known components such as olefins including, acrylates, methacrylates, styrene and its derivatives such as methyl acrylate, ethylacrylate, propyl acrylate, butyl acrylate, hexyl acrylate, methyl methacrylate, ethyl methacrylate, propyl methacrylate, butyl methacrylate, hexyl methacrylate, methyl styrene, and the like. Specific examples of nonionic monomers include styrene, alkyl substituted styrenes, halogenated styrenes, halogenated alkyl substituted styrenes and the like.

Illustrative examples of the nonionic diolefinc or diene monomers useful in the instant invention, include a number of known components as butadiene, substituted butadienes, for example, methyl butadiene, isoprene, mycerine, alkyl substituted isoprene, mixtures thereof and the like.

The copolymer resins formed from the above mentioned monomers are generally present in the toner composition in various effective amounts depending, for example, on the amount of the other components, and providing many of the objectives of the present invention are achievable. Generally, from about 70 to about 95 percent by weight of the copolymer resin is present in the toner composition, and preferably from about 75 to about 90 percent by weight. The proportion of the two monomers in the copolymer resin is from about 50 to about 95 weight percent of olefin and from about 5 to about 50 weight percent of diolefinc or diene.

Typical examples of specific colorants, preferably present in an effective amount of, for example, from about 3 to about 10 weight percent of toner include Paliogen Violet 5100 and 5890 (BASF), Normandy Magenta RD-2400 (Paul Uhlich), Permanent Violet VT2645 (Paul Uhlich), Heliogen Green L8730 (BASF),

Argyle Green XP-111-S (Paul Uhlich), Brilliant Green Toner GR 0991 (Paul Uhlich), Lithol Scarlet D3700 (BASF), Toluidine Red (Aldrich), Scarlet for Thermoplast NSD Red (Aldrich), Lithol Rubine Toner (Paul Uhlich), Lithol Scarlet 4440, NBD 3700 (BASF), Bon Red C (Dominion Color), Royal Brilliant Red RD-8192 (Paul Uhlich), Oracet Pink RF (Ciba Geigy), Paliogen Red 3340 and 3871K (BASF), Lithol Fast Scarlet L4300 (BASF), Heliogen Blue D6840, D7080, K7090, K6910 and L7020 (BASF), Sudan Blue OS (BASF), Neopen Blue FF4012 (BASF), PV Fast Blue B2G01 (American Hoechst), Irgalite Blue BCA (Ciba Geigy), Paliogen Blue 6470 (BASF), Sudan II, III and IV (Matheson, Coleman, Bell), Sudan Orange (Aldrich), Sudan Orange 220 (BASF), Paliogen Orange 3040 (BASF), Ortho Orange OR 2673 (Paul Uhlich), Paliogen Yellow 152 and 1560 (BASF), Lithol Fast Yellow 0991K (BASF), Paliotol Yellow 1840 (BASF), Novaperm Yellow FGL (Hoechst), Permanent Yellow YE 0305 (Paul Uhlich), Lumogen Yellow D0790 (BASF), Suco-Gelb L1250 (BASF), Suco-Yellow D1355 (BASF), Sico Fast Yellow D1165, D1355 and D1351 (BASF), Hostaperm Pink E (Hoechst), Fanal Pink D4830 (BASF), Cinquasia Magenta (DuPont), Paliogen Black L0084 (BASF), Pigment Black K801 (BASF) and carbon blacks such as REGAL 330? (Cabot), Carbon Black 5250 and 5750 (Columbian Chemicals), and the like.

Surfactants utilized are known and include, for example, nonionics surfactant such as polyvinyl alcohol, polyacrylic acid, methalose, methyl cellulose, ethyl cellulose, propyl cellulose, hydroxy ethyl cellulose, carboxy methylcellulose, polyoxyethylene cetyl ether, polyoxyethylene lauryl ether, polyoxyethylene octyl ether, polyoxyethylene octyphenyl ether, polyoxyethylene oleyl ether, polyoxyethylene sorbitan monolaurate, polyoxyethylene stearyl ether, polyoxyethylene nonylphenyl ether (available from GAF as Igepal CA-210, Igepal CA-520, Igepal CA-720, Igepal CO-890, Igepal CO-720, Igepal CO-290, Igepal CA-210, Antarax 890 and Antarax 897 available from Phone-Poulenc, dialkylphenoxy poly(ethyleneoxy)ethanol and the like. An effective concentration of the nonionic surfactant generally employed is, for example, from about 0.01 to about 10 percent by weight, and preferably from about 0.1 to about 5 percent by weight of monomers used to prepare the copolymer resin.

Examples of anionic surfactants selected for the preparation of toners and processes of the present invention are, for example, sodium dodecylsulfate (SDS), sodium dodecyl-benzenesulfate, sodium dodecylnaphthalenesulfate, dialkyl benzenealkyl, sulfates and sulfonates and the like. An effective concentration of the anionic surfactant generally employed is, for example, from about 0.01 to about 10 percent by weight, and preferably from about 0.1 to about 5 percent by weight of monomers used to prepare the copolymer resin.

Examples of the cationic surfactants selected for the toners and processes of the present invention are, for example, dialkyl benzenealkyl ammonium chloride, lauryl trimethyl ammonium chloride, alkylbenzyl methyl ammonium chloride, halide salts of quaternized polyoxyethylalkylamines, dodecylbenzyl triethyl ammonium chloride, MIRAPOL™ and AL-KAQUAT™ available from Alkaril Chemical Company, SANIZOL™, available from Kao Chemicals, and the like and mixtures thereof. An effective concentration of the cationic surfactant generally employed is,

for example, from about 0.01 to about 10 percent by weight and preferably from about 0.1 to about 5 percent by weight of monomers used to prepare the copolymer resin.

An effective concentration of a chain transfer agent that is generally employed is, for example, from about 0.005 to about 0.5 percent by weight, and preferably from about 0.01 to about 0.10 percent by weight of monomers, of for example, dodecanethiol, carbon tetrabromide and the like.

Illustrative examples of known free radical initiators that can be selected for the preparation of the toners include azo-type initiators such as 2-2'-azobis(dimethylvaleronitrile), azobis(isobutyronitrile), azobis(cyclohexane-nitrile), azobis(methyl-butyronitrile), mixtures thereof, and the like, peroxide initiators such as benzoyl peroxide, lauroyl peroxide, methyl ethyl ketone peroxide, isopropyl peroxy-carbonate, 2,5-dimethyl-2,5-bis(2-ethylhexanoyl-peroxy)hexane, di-tert-butyl peroxide, cumene hydroperoxide, dichlorobenzoyl peroxide, potassium persulfate, ammonium persulfate, sodium bisulfite, combination of potassium persulfate and sodium bisulfite, mixtures thereof, with the effective quantity of initiator being, for example, from about 0.1 percent to about 10 percent by weight of that of core monomer.

The aforementioned toner sized particles obtained from heating the statically bound aggregate composite particles of step (vii) of the toner process are optionally surface halogenated, partially or exhaustively, for example 100 percent, to convert olefinic double bonds by an electrophilic addition reaction in the surface polymer chain backbone and pendant groups into the corresponding halogenated hydrocarbon functionality. In many instances, surface halogenation of toner particles affords further control of the variety of rheological properties that may be obtained from the copolymer resins. Surface halogenation is accomplished with a gaseous mixture or liquid solution of an effective amount of from 0.01 to about 5 double bond molar equivalents of halogen gas or halogen liquid dissolved in water, or an organic solvent, for example, chlorine gas, liquid bromine, or crystalline iodine dissolved in a solvent, such as an aliphatic alcohol, like ethanol which does not dissolve or substantially alter the size or shape of the toner particles.

When more reactive halogens such as fluorine (F<sub>2</sub>) are used, an inert carrier gas, such as argon or nitrogen, may be selected as a diluent, for example, from about 0.1 to about 98 percent by volume of the inert gas relative to the reactive halogen gas, to moderate the extent of reaction, and the temperature and control corrosivity of the halogenation-encapsulation process.

A number of equally useful halogenating agents are known that afford equivalent reaction products with olefinic double bonds as the aforementioned diatomic halogens, for example as disclosed by House in "Modern Synthetic Reactions", W. A. Benjamin, Inc., 2nd Ed., Chapter 8, page 422, and references cited therein, the disclosure of which is incorporated in its entirety by reference.

The aggregate composite particles obtained from the heating step are subjected to optional halogenation, especially chlorination, by, for example, admixing the toner with an aqueous solution of the halogen. Halogens include chlorine, bromine, iodine, and fluorine, with chlorine being preferred. With fluorine, an aqueous solution is not utilized, rather there is selected fluorine with an inert atmosphere. Although it is not desired to

be limited by theory, it is believed that the halogen, especially the chlorine, adds across the double bonds of the toner resin particles to form carbon-halogen bonds. The aforementioned halogenation can be considered an addition reaction, that is, for example, the halogen reacts with, and diffuses into the toner resin, whereby a shell thereof is formed. The shell can be of various effective thicknesses; generally, however, the shell is of a thickness of from about 1 micron or less, and more specifically from about 0.1 to about 1 micron, in embodiments. Typical amounts of halogen consumed include, for example, from about 0.1 to about 1 gram of halogen per 100 grams of toner polymer resin. In an embodiment, the composite particles are admixed with a solution of water and chlorine, which solution has a pH of from about 2.0 to about 3.0, and preferably about 2.5. Specifically, about 150 grams of composite particles can be added in 300 milliliters of an alcohol, such as ethanol, to about 7.5 liters of a chlorine solution at a pH of between about 2.5 and about 3.0, resulting in a pH thereof of from about 2.6 to about 3.2 after about 20 minutes. Generally, from about 100 grams to about 200 grams of toner are admixed with from about 5 to about 10 liters of halogen solution, especially chlorine solution, which solution is comprised of water and halogen, it being noted that a fluorine solution is usually not selected as indicated herein. A sufficient amount of nonpolar composite particles and halogen solution are admixed to enable the formation of an effective shell.

The following examples are provided to further define various species of the present invention. These examples are intended to be illustrative only and are not intended to limit the scope of the present invention.

#### EXAMPLE I

A 9 micron in situ toner comprised of Hostaperm TM Pink E-21 pigment, poly(styrene butadiene) and outer resin surface of chlorinated poly(styrene butadiene).

A one liter stainless steel PARR TM reactor was charged with 400 grams of water, 88 grams of styrene, 4 grams of dodecanethiol, 2 grams of polyoxyethylene nonyl phenyl ether (Antarax 897, available from Rhone-Poulenc), 2 grams of sodium dodecylsulfate and 1.5 grams of potassium persulfate. Next was added 27 grams liquid butadiene at 5 degrees centigrade and the mixture pressurized to about 40 pounds per square inch with nitrogen gas. The mixture was then heated to 80 degrees centigrade for 6 hours, followed by cooling to room temperature to yield a latex comprised of about 40 percent by weight of solids comprised of nonpolar poly(styrene-butadiene) emulsion resin. A portion of this nonpolar olefinic emulsion resin was then washed, dried and characterized to display a glass transition temperature of about 45 degrees centigrade, and a number average molecular weight of 16,000 by Gel Permeation Chromatography (GPC) utilizing polystyrene standards. A one liter kettle was then charged with 200 grams of the aforementioned latex, 40 percent solids of poly(styrene-butadiene), 8 grams of a wet cake of Hostaperm TM Pink E-21 (50 percent solids in water) and the mixture homogenized using a Brinkman probe for 10 minutes at 4000 revolutions per minute. To this dispersion, was then added 1 gram dialkyl benzene alkyl ammonium chloride (Alkaquat TM, available from Alkaril Chemical Limited) resulting in flocculation of 65

5  
10  
15  
20  
25  
30  
35  
40  
45  
50  
55  
60  
65  
70  
75  
80  
85  
90  
95  
100  
105  
110  
115  
120  
125  
130  
135  
140  
145  
150  
155  
160  
165  
170  
175  
180  
185  
190  
195  
200  
205  
210  
215  
220  
225  
230  
235  
240  
245  
250  
255  
260  
265  
270  
275  
280  
285  
290  
295  
300  
305  
310  
315  
320  
325  
330  
335  
340  
345  
350  
355  
360  
365  
370  
375  
380  
385  
390  
395  
400  
405  
410  
415  
420  
425  
430  
435  
440  
445  
450  
455  
460  
465  
470  
475  
480  
485  
490  
495  
500  
505  
510  
515  
520  
525  
530  
535  
540  
545  
550  
555  
560  
565  
570  
575  
580  
585  
590  
595  
600  
605  
610  
615  
620  
625  
630  
635  
640  
645  
650  
655  
660  
665  
670  
675  
680  
685  
690  
695  
700  
705  
710  
715  
720  
725  
730  
735  
740  
745  
750  
755  
760  
765  
770  
775  
780  
785  
790  
795  
800  
805  
810  
815  
820  
825  
830  
835  
840  
845  
850  
855  
860  
865  
870  
875  
880  
885  
890  
895  
900  
905  
910  
915  
920  
925  
930  
935  
940  
945  
950  
955  
960  
965  
970  
975  
980  
985  
990  
995  
1000  
1005  
1010  
1015  
1020  
1025  
1030  
1035  
1040  
1045  
1050  
1055  
1060  
1065  
1070  
1075  
1080  
1085  
1090  
1095  
1100  
1105  
1110  
1115  
1120  
1125  
1130  
1135  
1140  
1145  
1150  
1155  
1160  
1165  
1170  
1175  
1180  
1185  
1190  
1195  
1200  
1205  
1210  
1215  
1220  
1225  
1230  
1235  
1240  
1245  
1250  
1255  
1260  
1265  
1270  
1275  
1280  
1285  
1290  
1295  
1300  
1305  
1310  
1315  
1320  
1325  
1330  
1335  
1340  
1345  
1350  
1355  
1360  
1365  
1370  
1375  
1380  
1385  
1390  
1395  
1400  
1405  
1410  
1415  
1420  
1425  
1430  
1435  
1440  
1445  
1450  
1455  
1460  
1465  
1470  
1475  
1480  
1485  
1490  
1495  
1500  
1505  
1510  
1515  
1520  
1525  
1530  
1535  
1540  
1545  
1550  
1555  
1560  
1565  
1570  
1575  
1580  
1585  
1590  
1595  
1600  
1605  
1610  
1615  
1620  
1625  
1630  
1635  
1640  
1645  
1650  
1655  
1660  
1665  
1670  
1675  
1680  
1685  
1690  
1695  
1700  
1705  
1710  
1715  
1720  
1725  
1730  
1735  
1740  
1745  
1750  
1755  
1760  
1765  
1770  
1775  
1780  
1785  
1790  
1795  
1800  
1805  
1810  
1815  
1820  
1825  
1830  
1835  
1840  
1845  
1850  
1855  
1860  
1865  
1870  
1875  
1880  
1885  
1890  
1895  
1900  
1905  
1910  
1915  
1920  
1925  
1930  
1935  
1940  
1945  
1950  
1955  
1960  
1965  
1970  
1975  
1980  
1985  
1990  
1995  
2000  
2005  
2010  
2015  
2020  
2025  
2030  
2035  
2040  
2045  
2050  
2055  
2060  
2065  
2070  
2075  
2080  
2085  
2090  
2095  
2100  
2105  
2110  
2115  
2120  
2125  
2130  
2135  
2140  
2145  
2150  
2155  
2160  
2165  
2170  
2175  
2180  
2185  
2190  
2195  
2200  
2205  
2210  
2215  
2220  
2225  
2230  
2235  
2240  
2245  
2250  
2255  
2260  
2265  
2270  
2275  
2280  
2285  
2290  
2295  
2300  
2305  
2310  
2315  
2320  
2325  
2330  
2335  
2340  
2345  
2350  
2355  
2360  
2365  
2370  
2375  
2380  
2385  
2390  
2395  
2400  
2405  
2410  
2415  
2420  
2425  
2430  
2435  
2440  
2445  
2450  
2455  
2460  
2465  
2470  
2475  
2480  
2485  
2490  
2495  
2500  
2505  
2510  
2515  
2520  
2525  
2530  
2535  
2540  
2545  
2550  
2555  
2560  
2565  
2570  
2575  
2580  
2585  
2590  
2595  
2600  
2605  
2610  
2615  
2620  
2625  
2630  
2635  
2640  
2645  
2650  
2655  
2660  
2665  
2670  
2675  
2680  
2685  
2690  
2695  
2700  
2705  
2710  
2715  
2720  
2725  
2730  
2735  
2740  
2745  
2750  
2755  
2760  
2765  
2770  
2775  
2780  
2785  
2790  
2795  
2800  
2805  
2810  
2815  
2820  
2825  
2830  
2835  
2840  
2845  
2850  
2855  
2860  
2865  
2870  
2875  
2880  
2885  
2890  
2895  
2900  
2905  
2910  
2915  
2920  
2925  
2930  
2935  
2940  
2945  
2950  
2955  
2960  
2965  
2970  
2975  
2980  
2985  
2990  
2995  
3000  
3005  
3010  
3015  
3020  
3025  
3030  
3035  
3040  
3045  
3050  
3055  
3060  
3065  
3070  
3075  
3080  
3085  
3090  
3095  
3100  
3105  
3110  
3115  
3120  
3125  
3130  
3135  
3140  
3145  
3150  
3155  
3160  
3165  
3170  
3175  
3180  
3185  
3190  
3195  
3200  
3205  
3210  
3215  
3220  
3225  
3230  
3235  
3240  
3245  
3250  
3255  
3260  
3265  
3270  
3275  
3280  
3285  
3290  
3295  
3300  
3305  
3310  
3315  
3320  
3325  
3330  
3335  
3340  
3345  
3350  
3355  
3360  
3365  
3370  
3375  
3380  
3385  
3390  
3395  
3400  
3405  
3410  
3415  
3420  
3425  
3430  
3435  
3440  
3445  
3450  
3455  
3460  
3465  
3470  
3475  
3480  
3485  
3490  
3495  
3500  
3505  
3510  
3515  
3520  
3525  
3530  
3535  
3540  
3545  
3550  
3555  
3560  
3565  
3570  
3575  
3580  
3585  
3590  
3595  
3600  
3605  
3610  
3615  
3620  
3625  
3630  
3635  
3640  
3645  
3650  
3655  
3660  
3665  
3670  
3675  
3680  
3685  
3690  
3695  
3700  
3705  
3710  
3715  
3720  
3725  
3730  
3735  
3740  
3745  
3750  
3755  
3760  
3765  
3770  
3775  
3780  
3785  
3790  
3795  
3800  
3805  
3810  
3815  
3820  
3825  
3830  
3835  
3840  
3845  
3850  
3855  
3860  
3865  
3870  
3875  
3880  
3885  
3890  
3895  
3900  
3905  
3910  
3915  
3920  
3925  
3930  
3935  
3940  
3945  
3950  
3955  
3960  
3965  
3970  
3975  
3980  
3985  
3990  
3995  
4000  
4005  
4010  
4015  
4020  
4025  
4030  
4035  
4040  
4045  
4050  
4055  
4060  
4065  
4070  
4075  
4080  
4085  
4090  
4095  
4100  
4105  
4110  
4115  
4120  
4125  
4130  
4135  
4140  
4145  
4150  
4155  
4160  
4165  
4170  
4175  
4180  
4185  
4190  
4195  
4200  
4205  
4210  
4215  
4220  
4225  
4230  
4235  
4240  
4245  
4250  
4255  
4260  
4265  
4270  
4275  
4280  
4285  
4290  
4295  
4300  
4305  
4310  
4315  
4320  
4325  
4330  
4335  
4340  
4345  
4350  
4355  
4360  
4365  
4370  
4375  
4380  
4385  
4390  
4395  
4400  
4405  
4410  
4415  
4420  
4425  
4430  
4435  
4440  
4445  
4450  
4455  
4460  
4465  
4470  
4475  
4480  
4485  
4490  
4495  
4500  
4505  
4510  
4515  
4520  
4525  
4530  
4535  
4540  
4545  
4550  
4555  
4560  
4565  
4570  
4575  
4580  
4585  
4590  
4595  
4600  
4605  
4610  
4615  
4620  
4625  
4630  
4635  
4640  
4645  
4650  
4655  
4660  
4665  
4670  
4675  
4680  
4685  
4690  
4695  
4700  
4705  
4710  
4715  
4720  
4725  
4730  
4735  
4740  
4745  
4750  
4755  
4760  
4765  
4770  
4775  
4780  
4785  
4790  
4795  
4800  
4805  
4810  
4815  
4820  
4825  
4830  
4835  
4840  
4845  
4850  
4855  
4860  
4865  
4870  
4875  
4880  
4885  
4890  
4895  
4900  
4905  
4910  
4915  
4920  
4925  
4930  
4935  
4940  
4945  
4950  
4955  
4960  
4965  
4970  
4975  
4980  
4985  
4990  
4995  
5000  
5005  
5010  
5015  
5020  
5025  
5030  
5035  
5040  
5045  
5050  
5055  
5060  
5065  
5070  
5075  
5080  
5085  
5090  
5095  
5100  
5105  
5110  
5115  
5120  
5125  
5130  
5135  
5140  
5145  
5150  
5155  
5160  
5165  
5170  
5175  
5180  
5185  
5190  
5195  
5200  
5205  
5210  
5215  
5220  
5225  
5230  
5235  
5240  
5245  
5250  
5255  
5260  
5265  
5270  
5275  
5280  
5285  
5290  
5295  
5300  
5305  
5310  
5315  
5320  
5325  
5330  
5335  
5340  
5345  
5350  
5355  
5360  
5365  
5370  
5375  
5380  
5385  
5390  
5395  
5400  
5405  
5410  
5415  
5420  
5425  
5430  
5435  
5440  
5445  
5450  
5455  
5460  
5465  
5470  
5475  
5480  
5485  
5490  
5495  
5500  
5505  
5510  
5515  
5520  
5525  
5530  
5535  
5540  
5545  
5550  
5555  
5560  
5565  
5570  
5575  
5580  
5585  
5590  
5595  
5600  
5605  
5610  
5615  
5620  
5625  
5630  
5635  
5640  
5645  
5650  
5655  
5660  
5665  
5670  
5675  
5680  
5685  
5690  
5695  
5700  
5705  
5710  
5715  
5720  
5725  
5730  
5735  
5740  
5745  
5750  
5755  
5760  
5765  
5770  
5775  
5780  
5785  
5790  
5795  
5800  
5805  
5810  
5815  
5820  
5825  
5830  
5835  
5840  
5845  
5850  
5855  
5860  
5865  
5870  
5875  
5880  
5885  
5890  
5895  
5900  
5905  
5910  
5915  
5920  
5925  
5930  
5935  
5940  
5945  
5950  
5955  
5960  
5965  
5970  
5975  
5980  
5985  
5990  
5995  
6000  
6005  
6010  
6015  
6020  
6025  
6030  
6035  
6040  
6045  
6050  
6055  
6060  
6065  
6070  
6075  
6080  
6085  
6090  
6095  
6100  
6105  
6110  
6115  
6120  
6125  
6130  
6135  
6140  
6145  
6150  
6155  
6160  
6165  
6170  
6175  
6180  
6185  
6190  
6195  
6200  
6205  
6210  
6215  
6220  
6225  
6230  
6235  
6240  
6245  
6250  
6255  
6260  
6265  
6270  
6275  
6280  
6285  
6290  
6295  
6300  
6305  
6310  
6315  
6320  
6325  
6330  
6335  
6340  
6345  
6350  
6355  
6360  
6365  
6370  
6375  
6380  
6385  
6390  
6395  
6400  
6405  
6410  
6415  
6420  
6425  
6430  
6435  
6440  
6445  
6450  
6455  
6460  
6465  
6470  
6475  
6480  
6485  
6490  
6495  
6500  
6505  
6510  
6515  
6520  
6525  
6530  
6535  
6540  
6545  
6550  
6555  
6560  
6565  
6570  
6575  
6580  
6585  
6590  
6595  
6600  
6605  
6610  
6615  
6620  
6625  
6630  
6635  
6640  
6645  
6650  
6655  
6660  
6665  
6670  
6675  
6680  
6685  
6690  
6695  
6700  
6705  
6710  
6715  
6720  
6725  
6730  
6735  
6740  
6745  
6750  
6755  
6760  
6765  
6770  
6775  
6780  
6785  
6790  
6795  
6800  
6805  
6810  
6815  
6820  
6825  
6830  
6835  
6840  
6845  
6850  
6855  
6860  
6865  
6870  
6875  
6880  
6885  
6890  
6895  
6900  
6905  
6910  
6915  
6920  
6925  
6930  
6935  
6940  
6945  
6950  
6955  
6960  
6965  
6970  
6975  
6980  
6985  
6990  
6995  
7000  
7005  
7010  
7015  
7020  
7025  
7030  
7035  
7040  
7045  
7050  
7055  
7060  
7065  
7070  
7075  
7080  
7085  
7090  
7095  
7100  
7105  
7110  
7115  
7120  
7125  
7130  
7135  
7140  
7145  
7150  
7155  
7160  
7165  
7170  
7175  
7180  
7185  
7190  
7195  
7200  
7205  
7210  
7215  
7220  
7225  
7230  
7235  
7240  
7245  
7250  
7255  
7260  
7265  
7270  
7275  
7280  
7285  
7290  
7295  
7300  
7305  
7310  
7315  
7320  
7325  
7330  
7335  
7340  
7345  
7350  
7355  
7360  
7365  
7370  
7375  
7380  
7385  
7390  
7395  
7400  
7405  
7410  
7415  
7420  
7425  
7430  
7435  
7440  
7445  
7450  
7455  
7460  
7465  
7470  
7475  
7480  
7485  
7490  
7495  
7500  
7505  
7510  
7515  
7520  
7525  
7530  
7535  
7540  
7545  
7550  
7555  
7560  
7565  
7570  
7575  
7580  
7585  
7590  
7595  
7600  
7605  
7610  
7615  
7620  
7625  
7630  
7635  
7640  
7645  
7650  
7655  
7660  
7665  
7670  
7675  
7680  
7685  
7690  
7695  
7700  
7705  
7710  
7715  
7720  
7725  
7730  
7735  
7740  
7745  
7750  
7755  
7760  
7765  
7770  
7775  
7780  
7785  
7790  
7795  
7800  
7805  
7810  
7815  
7820  
7825  
7830  
7835  
7840  
7845  
7850  
7855  
7860  
7865  
7870  
7875  
7880  
7885  
7890  
7895  
7900  
7905  
7910  
7915  
7920  
7925  
7930  
7935  
7940  
7945  
7950  
7955  
7960  
7965  
7970  
7975  
7980  
7985  
7990  
7995  
8000  
8005  
8010  
8015  
8020  
8025  
8030  
8035  
8040  
8045  
8050  
8055  
8060  
8065  
8070  
8075  
8080  
8085  
8090  
8095  
8100  
8105  
8110  
8115  
8120  
8125  
8130  
8135  
8140  
8145  
8150  
8155  
8160  
8165  
8170  
8175  
8180  
8185  
8190  
8195  
8200  
8205  
8210  
8215  
8220  
8225  
8230  
8235  
8240  
8245  
8250  
8255  
8260  
8265  
8270  
8275  
8280  
8285  
8290  
8295  
8300  
8305  
8310  
8315  
8320  
8325  
8330  
8335  
8340  
8345  
8350  
8355  
8360  
8365  
8370  
8375  
8380  
8385  
8390  
8395  
8400  
8405  
8410  
8415  
8420  
8425  
8430  
8435  
8440  
8445  
8450  
8455  
8460  
8465  
8470  
8475  
8480  
8485  
8490  
8495  
8500  
8505  
8510  
8515  
8520  
8525  
8530  
8535  
8540  
8545  
8550  
8555  
8560  
8565  
8570  
8575  
8580  
8585  
8590  
8595  
8600  
8605  
8610  
8615  
8620  
8625  
8630  
8635  
8640  
8645  
8650  
8655  
8660  
8665  
8670  
8675  
8680  
8685  
8690  
8695  
8700  
8705  
8710  
8715  
8720  
8725  
8730  
8735  
8740  
8745  
8750  
8755<br

duration of 10 minutes at 4000 revolutions per minute. To this dispersion, was then added 1 gram dialkyl benzene alkyl ammonium chloride (Alkaquat, available from Alkaril Chemical Limited) resulting in flocculation of pigment and nonpolar emulsion resin particles. The flocculated material was then emulsified utilizing a Brinkman probe for 10 minutes at 8000 revolutions per minute resulting in a dispersion of statically bound aggregates of pigment and nonpolar olefinic resin emulsion particles. When a sample of the dispersion was viewed under a microscope, the aggregate sizes were observed to range from submicron to about 5 microns in diameter. The dispersion was stirred for 14 hours and then heated for 8 hours at 70 degrees centigrade, and then cooled to 5 degrees centigrade using an ice-water bath mixture. To this was then bubbled chlorine gas until a pH of about 3 was obtained, and then stirring was continued for an additional 30 minutes. The toner particles were then repeatedly washed with warm water (60 to 70 degrees centigrade) and filtered off. The wet toner cake was then fluidized in a Aeromatic AG TM bed drier operated at 50 degrees centigrade for 3 hours. The dry toner particles (76 grams, 91% yield) were measured by a Coulter counter to have a volume average diameter particle size of 9 microns.

#### EXAMPLE IV

A 5 micron in situ toner comprised of Hostaperm TM Pink E-21 pigment, poly(styrene butadiene) and outer resin surface of chlorinated poly(styrene butadiene) was prepared as follows:

A one liter stainless steel PARR TM reactor was charged with 400 grams of water, 88 grams of styrene, 4 grams of dodecanethiol, 2 grams of polyoxyethylene nonyl phenyl ether (Antarax 897, available from Rhone-Poulenc), 2 grams of sodium dodecylsulfate and 1.5 grams of potassium persulfate. To this was then added 17 grams liquid butadiene at 5 degrees centigrade, and the mixture pressurized to about 40 pounds per square inch with nitrogen gas. The mixture was then heated to 80 degrees centigrade for 6 hours, followed by cooling to room temperature to yield a latex comprised of about 40 percent nonpolar poly(styrene-butadiene) emulsion resin. A portion of this nonpolar olefinic emulsion resin was then washed, dried and characterized as having a glass transition temperature of about 45 degrees centigrade, and a number average molecular weight of 16,000 by GPC utilizing polystyrene standards. A one liter kettle was then charged with 200 grams of the aforementioned latex (40 percent solid of poly-(styrene-butadiene), 8 grams of a wet cake of Hostaperm TM Pink E-21 (50 percent solids in water) and the mixture homogenized using a Brinkman probe for a duration of 55 10 minutes and at a speed of 4000 revolution per minute. To this dispersion was then added 1 gram dialkyl benzene alkyl ammonium chloride (Alkaquat, available from Alkaril Chemical Limited) resulting in flocculation of pigment and nonpolar emulsion particles. The 60 flocculated material was then emulsified utilizing a Brinkman probe for 10 minutes at 8000 revolutions per minute resulting in a dispersion of statically bound aggregates of pigment and nonpolar olefinic version emulsion particles. When a sample of the dispersion was viewed under a microscope, the aggregate sizes were observed to range from submicron to about 5 microns in diameter. The dispersion was then heated for a duration

of 12 hours at 80 degrees centigrade, and then cooled to 5 degrees centigrade using an ice-water bath mixture. To this was then bubbled chlorine gas until a pH of about 3 was obtained, and then stirring was continued for an additional 30 minutes. The toner particles were then repeatedly washed with warm water (60 to 70 degrees centigrade) and filtered. The wet toner cake was then fluidized in a Aeromatic AG TM bed drier operated at 50 degrees centigrade for 3 hours. The dry toner particles (76 grams, 91% yield) were measured by a Coulter counter to have a volume average diameter particle size of 9 microns.

#### EXAMPLE V

A 7.5 micron in situ toner comprised of Heliogen TM blue pigment, poly(styrene butadiene) and outer resin surface of chlorinated poly(styrene butadiene) was prepared as follows:

A mixture of 4 grams of Heliogen TM Blue pigment and one gram of dialkyl benzene alkyl ammonium chloride (Alkaquat, available from Alkaril Chemicals Limited) was sonicated for 30 minutes using a Branson 750 ultrasonicator. The resulting pigment dispersion was added to 200 grams of the aforementioned latex prepared in Example 1 (40 percent solids of poly(styrene-butadiene)) in a one liter kettle. The mixture was then homogenized using a Brinkman probe for 10 minutes at 4000 revolutions per minute. To this dispersion, was then added 1 gram dialkyl benzenealkyl ammonium chloride (Alkaquat, available from Alkaril Chemical Limited) resulting in a flocculation of pigment and nonpolar emulsion particles. The flocculated material was then homogenized utilizing a Brinkman probe for a duration of 10 minutes and at a speed of 8000 revolution per minute resulting in a dispersion of statically bounded aggregates of pigment and nonpolar olefinic emulsion. When a 1 gram sample of the dispersion was viewed under a microscope, the aggregate sizes were observed to range from submicron to about 6 microns in diameter. The dispersion was stirred for 14 hours and then heated for a duration of 10 hours at 75 degrees centigrade, and then cooled to 5 degrees centigrade using an ice-water bath mixture. To this was then bubbled chlorine gas until a pH of about 3 was obtained, and then stirring was continued for an additional 30 minutes. The toner particles were then repeatedly washed with warm water (60 to 70 degrees centigrade) and filtered off. The wet toner cake was then fluidized in a Aeromatic AG TM bed drier operated at 50 degrees centigrade and for a duration of 3 hours. The dry toner particles (76 grams, 91% yield) were then measured by a Coulter counter to display a volume average diameter particle size of 7.5 microns and geometric size distribution of 1.53.

#### EXAMPLE VI

A 9.2 micron in situ toner comprised of Heliogen TM blue pigment, poly(styrene butadiene) and outer resin surface of chlorinated poly(styrene butadiene) was prepared as follows:

A mixture of 4 grams of Heliogen TM Blue pigment and one gram of dialkyl benzene alkyl ammonium chloride (Alkaquat, available from Alkaril Chemicals Limited) was sonicated for 30 minutes using a Branson 750 ultrasonicator. The resulting pigment dispersion was added to 200 grams of the aforementioned latex prepared in Example 1 (40 percent solid of poly(styrene-butadiene)) in a one liter kettle. The mixture was then

homogenized using a Brinkman probe for 10 minutes at 4000 revolutions per minute. To this dispersion, was then added 1 gram dialkyl benzene alkyl ammonium chloride (Alkaquat, available from Alkaril Chemical Limited) resulting in a flocculation of pigment and nonpolar emulsion particles. The flocculents were then homogenized utilizing a Brinkman probe for a duration of 10 minutes and at a speed of 8000 revolution per minute resulting in a dispersion of statically bounded aggregates of pigment and nonpolar olefinic emulsion. When a sample of the dispersion was viewed under a microscope, the aggregate sizes were observed to range from submicron to about 6 microns in diameter. The dispersion was stirred for 14 hours and then heated for a duration of 12 hours at 80 degrees centigrade, and then cooled to 5 degrees centigrade using an ice-water bath mixture. To this was then bubbled chlorine gas until a pH of about 3 was obtained, and then stirring was continued for an additional 30 minutes. The toner particles were then repeatedly washed with warm water (60 to 70 degrees centigrade) and filtered off. The wet toner cake was then fluidized in a Aeromatic Ag TM bed drier operated at 50 degrees centigrade and for a duration of 3 hours. The dry toner particles (70 grams, 83% yield) were then measured by a Coulter counter to display a 25 volume average diameter particle size of 9.2 microns and geometric size distribution of 1.47.

#### EXAMPLE VII

A 9.5 micron in situ toner comprised of Hostaperm TM Regal 330 pigment, poly(styrene butadiene) and outer resin surface of chlorinated poly(styrene butadiene) was prepared as follows:

A one liter stainless steel PARR TM reactor was charged with 300 grams of water, 176 grams of styrene, 35 grams of dodecanethiol, 3 grams of polyoxyethylene nonyl phenyl ether (Antarax 897, available from Rhone-Poulenc), 4.5 grams of sodium dodecylsulfate and 2 grams of potassium persulfate. To this was then added 24 grams of liquid butadiene at 5 degrees centigrade, and the mixture pressurized to about 40 pounds per square inch with nitrogen gas. The mixture was then heated to 70 degrees centigrade for 8 hours, followed by cooling to room temperature to yield a latex comprised of about 40 percent by weight of solids comprised of 45 nonpolar poly(styrene-butadiene) emulsion resin. A portion of this nonpolar olefinic emulsion resin was then washed, dried and characterized as having a glass transition temperature of about 45 degrees centigrade, and a number average molecular weight of 33,100 by GPC 50 utilizing polystyrene standards. A one liter kettle was then charged with 200 grams of the aforementioned latex (40 percent solid of poly-(styrene-butadiene)), 8 grams of a wet cake of Hostaperm TM Pink E-21 (50 percent solids in water) and the mixture homogenized using a Brinkman probe for a duration of 10 minutes and at a speed of 4000 revolution per minute. To this dispersion, was then added 1 gram dialkyl benzene alkyl ammonium chloride (Alkaquat TM, available from Alkaril Chemical Limited) resulting in a flocculation of pigment and nonpolar emulsion resin particles. The flocculated particles were then homogenized with a Brinkman probe for a duration of 10 minutes and at a speed of 8000 revolution per minute resulting in a dispersion of statically bounded aggregates of pigment and nonpolar olefinic emulsion. When a sample of the dispersion was viewed under a microscope, the aggregate sizes were observed to range from submicron to about 5 microns in

diameter. The dispersion was stirred for 14 hours and then heated for a duration of 12 hours at 80 degrees centigrade, and then cooled to 5 degrees centigrade using an ice-water bath mixture. To this was then bubbled chlorine gas until a pH of about 3 was obtained, and then stirring was continued for an additional 30 minutes. The toner particles were then repeatedly washed with warm water (60 to 70 degrees centigrade) and filtered off. The wet toner cake was then fluidized in an Aeromatic AG TM bed drier operated at 50 degrees centigrade and for a duration of 3 hours. The dry toner particles (74 grams, 88% yield) were then measured by a Coulter counter to display a volume average diameter particle size of 9.5 microns and geometric size distribution of 1.41.

Other modifications of the present invention may occur to those skilled in the art subsequent to a review of the present application, and these modifications are intended to be included within the scope of the present invention.

What is claimed is:

1. A process for the preparation of a toner composition comprising the steps of:

- (i) preparing a latex emulsion by agitating in water a mixture of a nonionic surfactant, an anionic surfactant, a first nonpolar olefinic monomer, a second nonpolar diolefinic monomer, a free radical initiator and a chain transfer agent;
- (ii) polymerizing the latex emulsion mixture by heating from ambient temperature to about 80° C. to form nonpolar olefinic emulsion resin particles of volume average diameter from about 5 nanometers to about 500 nanometers;
- (iii) diluting the nonpolar olefinic emulsion resin particle mixture with water;
- (iv) adding to the diluted resin particle mixture a colorant or pigment particles and optionally dispersing the resulting mixture with a homogenizer;
- (v) adding a cationic surfactant to flocculate the colorant or pigment particles to the surface of the emulsion resin particles;
- (vi) homogenizing the flocculated mixture at high shear to form statically bound aggregated composite particles with a volume average diameter of less than or equal to about 5 microns;
- (vii) heating the statically bound aggregate composite particles to form nonpolar toner sized particles;
- (viii) optionally halogenating the nonpolar toner sized particles to form nonpolar toner sized particles having a halopolymer resin outer surface or encapsulating shell; and
- (ix) isolating the nonpolar toner sized composite particles.

2. A process in accordance with claim 1 wherein the adding of colorant or pigment particles to the diluted particles of step (iv) is accomplished at a temperature of from about 25° C. to about 125° C.

3. A process in accordance with claim 1 wherein the optional dispersion of step (iv) is accomplished by homogenizing at from about 1000 revolution per minute to about 10,000 revolution per minute and at a temperature of from about 25° C. to about 35° C.

4. A process in accordance with claim 1 wherein the optional halogenation of step (viii) of the resin outer surface of nonpolar toner sized composite particles is accomplished with chlorine gas, liquid bromine or aqueous sodium hypochlorite at from about 5 to about 40 degrees centigrade.

5. A process in accordance with claim 1 wherein the nonpolar olefinic emulsion resin formed in step (ii) is selected from the group consisting of poly(styrene-butadiene), poly(para-methyl styrene-butadiene), poly(-meta-methyl styrene-butadiene), poly(alpha-methylstyrene-butadiene), poly(methylmethacrylate-butadiene), poly(ethylmethacrylate-butadiene), poly(propylmethacrylate-butadiene), poly(butylmethacrylate-butadiene), poly(methylacrylate-butadiene), poly(ethylacrylate-butadiene), poly(propylacrylate-butadiene), poly(butylacrylate-butadiene), poly(styrene-isoprene), poly(-para-methyl styrene-isoprene), poly(meta-methyl styrene-isoprene), poly(alpha-methylstyrene-isoprene), poly(methylmethacrylate-isoprene), poly(ethylmethacrylate-isoprene), poly(propylmethacrylate-isoprene), poly(butylmethacrylate-isoprene), poly(methylacrylate-isoprene), poly(ethylacrylate-isoprene), poly(propylacrylate-isoprene), and poly(butylacrylate-isoprene).

6. A process in accordance with claim 1 wherein the nonpolar olefinic emulsion resin formed in step (ii) is poly(styrene-butadiene).

7. A process in accordance with claim 1 wherein the nonionic surfactant is selected from the group consisting of polyvinyl alcohol, methalose, methyl cellulose, ethyl cellulose, propyl cellulose, hydroxy ethyl cellulose, carboxy methylcellulose, polyoxyethylene cetyl ether, polyoxyethylene lauryl ether, polyoxyethylene octyl ether, polyoxyethylene octyphenyl ether, polyoxyethylene oleyl ether, polyoxyethylene sorbitan monolaurate, polyoxyethylene stearyl ether, polyoxyethylene nonylphenyl ether, and dialkylphenoxy poly(ethyleneoxy)ethanol.

8. A process in accordance with claim 1 wherein the anionic surfactant is selected from the group consisting of sodium dodecylsulfate, sodium dodecylbenzenesulfate and sodium dodecylnaphthalenesulfate.

9. A process in accordance with claim 1 wherein the cationic surfactant is a quaternary ammonium salt.

10. A process in accordance with claim 1 wherein the pigment is carbon black, magnetite, or mixtures thereof; cyan, yellow, magenta, or mixtures thereof; or red, green, blue, brown, or mixtures thereof.

11. A process in accordance with claim 1 wherein the nonpolar olefinic resin particles formed in step (ii) are from about 10 to 500 nanometers in diameter.

12. A process in accordance with claim 1 wherein the pigment particles added in step (iv) are from about 10 to 300 nanometers in volume average diameter.

13. A process in accordance with claim 1 wherein the toner particles isolated in step (ix) are from about 3 to 15 micrometers in diameter.

14. A process in accordance with claim 1 wherein the statically bound aggregate particles formed in step (iv) are from about 0.5 to about 10 micrometers in diameter.

15. A process in accordance with claim 1 wherein the nonionic surfactant concentration is about 0.1 to about 5 weight percent of the monomer content in the aqueous nonpolar olefin mixture of step (i).

16. A process in accordance with claim 1 wherein the anionic surfactant concentration is about 0.1 to about 5 weight percent of the monomer content in the aqueous nonpolar olefin mixture of step (i).

17. A process in accordance with claim 1 wherein the toner particles isolated in step (ix) have a geometric size distribution of from about 1.2 to about 1.6.

18. A process in accordance with claim 1 wherein the cationic surfactant concentration is about 0.1 to about 5

weight percent of the monomer content of the aqueous nonpolar olefin mixture of step (i).

19. A process in accordance with claim 1 wherein there is added to the surface of the isolated toner particles surface additives of metal salts, metal salts of fatty acids, silicas, or mixtures thereof, in an amount of from about 0.1 to about 10 weight percent of the toner particles.

20. A toner composition comprising composite particles comprised of pigment particles and nonpolar olefinic resin particles wherein the outer resin surface of the composite particles is a chlorinated nonpolar resin.

21. A toner composition in accordance with claim 20 wherein the toner particle size is about 3 to about 15 microns in volume average diameter.

22. A toner composition in accordance with claim 20 wherein the pigment is carbon black, magnetite, or mixtures thereof; cyan, yellow, magenta, or mixtures thereof; or red, green, blue, brown, or mixtures thereof.

23. A toner composition in accordance with claim 20 wherein the nonpolar olefinic resin is poly(styrene-butadiene) and the chlorinated nonpolar resin is poly(styrene-butadiene-dichlorobutene).

24. A toner composition in accordance with claim 20 wherein the pigment particles are from about 10 to 300 nanometers volume average diameter.

25. A toner composition in accordance with claim 20 wherein the composite particles are from about 3 to 15 micrometers in volume average diameter.

26. A toner composition in accordance with claim 20 wherein the composite particles are from about 3 to 7 micrometers in volume average diameter.

27. A toner composition in accordance with claim 20 wherein the composite particles comprised of pigment particles and nonpolar olefinic resin particles are reacted with a halogen to afford composite particles comprised of pigment particles and nonpolar olefinic resin particles wherein the outer resin surface of the composite particles is a chlorinated nonpolar resin.

28. A toner composition in accordance with claim 20 wherein the composite particles comprised of pigment particles and monopolar olefinic resin particles has a glass transition temperature of about 40° to 55° C., and wherein the chlorinated nonpolar resin on the outer surface of the composite particles has a glass transition temperature of about 55° to 65° C.

29. A toner composition in accordance with claim 20 having gloss of from about 45 to about 85 gloss units and a projection efficiency of from about 75 to about 95 percent.

30. A process in accordance with claim 1 wherein diluting the nonpolar olefinic emulsion resin particle mixture of step (iii) is accomplished with water from about 50% solids to about 15% solids; adding a colorant or pigment particles to the diluted resin particle mixture of step (iv) is accomplished with from about 3 percent to about 15 percent colorant or pigment particles by weight of resin particles and optionally dispersing the resulting mixture with a homogenizer; heating the statically bound aggregate composite particles of step (vii) is accomplished at about 60 to about 95 degrees centigrade and from about 60 minutes to about 600 minutes to form nonpolar toner sized particles of from about 3 microns to about 9 microns in volume average diameter; and isolating the nonpolar toner sized composite particles of step (ix) is accomplished by washing, filtering and drying to afford a nonpolar composite toner particle composition.

\* \* \* \* \*